



US006524439B2

(12) **United States Patent**  
**Chen et al.**

(10) **Patent No.:** **US 6,524,439 B2**  
(b4) **Date of Patent:** **Feb. 25, 2003**

(54) **MANUFACTURE OF PAPER AND PAPERBOARD**

(75) Inventors: **Gordon Cheng I. Chen**, Chesapeake, VA (US); **Gary Peter Richardson**, Bradford (GB)

(73) Assignee: **Ciba Specialty Chemicals Water Treatments Ltd.**, Bradford (GB)

(\*) Notice: Subject to any disclaimer, the term of this patent is extended or adjusted under 35 U.S.C. 154(b) by 0 days.

(21) Appl. No.: **09/974,930**

(22) Filed: **Oct. 10, 2001**

(65) **Prior Publication Data**

US 2002/0066540 A1 Jun. 6, 2002

**Related U.S. Application Data**

(60) Provisional application No. 60/240,635, filed on Oct. 16, 2000.

(51) **Int. Cl.**<sup>7</sup> ..... **D21H 21/10**

(52) **U.S. Cl.** ..... **162/168.1; 162/181.6; 162/181.8; 162/182.1; 162/183.3; 162/183**

(58) **Field of Search** ..... 162/164.1, 168.1, 162/168.2, 168.3, 183, 181.1, 181.6, 181.8

(56) **References Cited**

**U.S. PATENT DOCUMENTS**

|             |           |                 |       |            |
|-------------|-----------|-----------------|-------|------------|
| 4,021,364 A | 5/1977    | Speiser et al.  | ..... | 252/316    |
| 4,388,150 A | 6/1983    | Sunden et al.   | ..... | 162/175    |
| 4,521,317 A | 6/1985    | Candau et al.   | ..... | 252/8.55   |
| 4,681,912 A | 7/1987    | Durand et al.   | ..... | 524/827    |
| 5,167,766 A | * 12/1992 | Honig et al.    | ..... | 162/164.1  |
| 5,176,891 A | 1/1993    | Rushmere        | ..... | 423/328.1  |
| 5,393,381 A | 2/1995    | Hund et al.     | ..... | 162/168.3  |
| 5,431,783 A | * 7/1995  | Honig           | ..... | 162/168.2  |
| 5,482,693 A | 1/1996    | Rushmere et al. | ..... | 423/328.1  |
| 5,501,774 A | * 3/1996  | Burke           | ..... | 162/181.67 |
| 5,584,966 A | 12/1996   | Moffett         | ..... | 162/168.1  |

5,676,796 A \* 10/1997 Cutts ..... 162/168.3  
5,882,525 A 3/1999 Neff et al. ..... 210/735  
6,007,679 A 12/1999 Nagarajan et al. ..... 162/168.3  
6,103,064 A \* 8/2000 Asplund et al. ..... 162/181.6

**FOREIGN PATENT DOCUMENTS**

|    |          |         |
|----|----------|---------|
| EP | 0235893  | 9/1987  |
| EP | 0308752  | 3/1989  |
| EP | 0335575  | 10/1989 |
| EP | 0462365  | 12/1991 |
| EP | 0484617  | 5/1992  |
| EP | 0485124  | 5/1992  |
| GB | 2161492  | 1/1986  |
| WO | 86/00100 | 1/1986  |
| WO | 97/33040 | 9/1997  |
| WO | 97/33041 | 9/1997  |
| WO | 98/29604 | 7/1998  |
| WO | 99/16708 | 4/1999  |
| WO | 01/34908 | 5/2001  |

**OTHER PUBLICATIONS**

S. Atik et al., *J. Am. Chem. Soc.* (1981), vol. 103, pp. 4279-4280.

Y. Huang et al., *Makromol. Chem.* vol. 186, pp. 273-281, (1985).

Stoffer et al., *J. Dispersion Sci. and Tech.*, vol. 1, No. 1, (1980), p. 37.

\* cited by examiner

*Primary Examiner*—Peter Chin

(74) *Attorney, Agent, or Firm*—David R. Crichton

(57) **ABSTRACT**

According to the present invention a process is provided for making paper or paper board comprising forming a cellulosic suspension, flocculating the suspension, draining the suspension on a screen to form a sheet and then drying the sheet, characterised in that the suspension is flocculated using a flocculation system comprising a siliceous material and organic microparticles which have an unswollen particle diameter of less than 750 nanometers.

**27 Claims, 3 Drawing Sheets**

Figure 1



Figure 2



Figure 3



## MANUFACTURE OF PAPER AND PAPERBOARD

This application claims benefit of U.S. Provisional Application No. 60/240,635 filed Oct. 16, 2000.

This invention relates to processes of making paper and paperboard from a cellulosic stock, employing a novel flocculating system.

During the manufacture of paper and paper board a cellulosic thin stock is drained on a moving screen (often referred to as a machine wire) to form a sheet which is then dried. It is well known to apply water soluble polymers to the cellulosic suspension in order to effect flocculation of the cellulosic solids and enhance drainage on the moving screen.

In order to increase output of paper many modern paper making machines operate at higher speeds. As a consequence of increased machine speeds a great deal of emphasis has been placed on drainage and retention systems that provide increased drainage. However, it is known that increasing the molecular weight of a polymeric retention aid which is added immediately prior to drainage will tend to increase the rate of drainage but damage formation. It is difficult to obtain the optimum balance of retention, drainage, drying and formation by adding a single polymeric retention aid and it is therefore common practice to add two separate materials in sequence.

EP-A-235893 provides a process wherein a water soluble substantially linear cationic polymer is applied to the paper making stock prior to a shear stage and then reflocculating by introducing bentonite after that shear stage. This process provides enhanced drainage and also good formation and retention. This process which is commercialised by Ciba Specialty Chemicals under the Hydrocol® trade mark has proved successful for more than a decade.

More recently there have been various attempts to provide variations on this theme by making minor modifications to one or more of the components.

U.S. Pat. No. 5,393,381 describes a process in which a process of making paper or board by adding a water soluble branched cationic polyacrylamide and a bentonite to the fibrous suspension of pulp. The branched cationic polyacrylamide is prepared by polymerising a mixture of acrylamide, cationic monomer, branching agent and chain transfer agent by solution polymerisation.

U.S. Pat. No. 5,882,525 describes a process in which a cationic branched water soluble polymer with a solubility quotient greater than about 30% is applied to a dispersion of suspended solids, e.g. a paper making stock, in order to release water. The cationic branched water soluble polymer is prepared from similar ingredients to U.S. Pat. No. 5,393,381 i.e. by polymerising a mixture of acrylamide, cationic monomer, branching agent and chain transfer agent.

In WO-A-9829604 a process of making paper is described in which a cationic polymeric retention aid is added to a cellulosic suspension to form flocs, mechanically degrading the flocs and then reflocculating the suspension by adding a solution of a second anionic polymeric retention aid. The anionic polymeric retention aid is a branched polymer which is characterised by having a rheological oscillation value of tan delta at 0.005 Hz of above 0.7 or by having a deionised SLV viscosity number which is at least three times the salted SLV viscosity number of the corresponding polymer made in the absence of branching agent. The process provided significant improvements in the combination of retention and formation by comparison to the earlier prior art processes.

EP-A-308752 describes a method of making paper in which a low molecular weight cationic organic polymer is added to the furnish and then a colloidal silica and a high molecular weight charged acrylamide copolymer of molecular weight at least 500,000. The description of the high molecular weight polymers indicates that they are linear polymers.

EP-A-462365 describes a method of making paper which comprises adding to an aqueous paper furnish ionic, organic microparticles which have an unswollen particle diameter of less than 750 nanometers if cross-linked and less than 60 nanometers if non-cross-linked and water-insoluble and have an anionicity of at least 1%, but at least 5% if cross-linked, anionic and used as the sole retention additive. The process is said to result in significant increase in fibre retention and improvements in drainage and formation.

EP-484617 describes a composition comprising cross-linked anionic or amphoteric, organic polymeric microparticles, said microparticles having an unswollen number average particle size diameter of less than 0.75 microns, a solution viscosity of at least 1.1 mPa.s and a cross-linking agent content of above 4 molar parts per million, based on the monomeric units and an ionicity of at least 5.0%. The polymers are described as being useful for a wide range of solid-liquid separation operations and specifically said to increase the drainage rates paper making.

However, there still exists a need to further enhance paper making processes by further improving drainage, retention and formation. Furthermore there also exists the need for providing a more effective flocculation system for making highly filled paper.

## BRIEF DESCRIPTION OF DRAWINGS

FIG. 1 is a graph retention versus dosage for various systems.

FIG. 2 is a graph showing ash retention versus dosage for various systems.

FIG. 3 is a graph showing drainage versus dosage for various systems.

According to the present invention a process is provided for making paper or paper board comprising forming a cellulosic suspension, flocculating the suspension, draining the suspension on a screen to form a sheet and then drying the sheet, characterised in that the suspension is flocculated using a flocculation system comprising a siliceous material and organic microparticles which have an unswollen particle diameter of less than 750 nanometers.

The microparticles may be prepared according to any suitable technique documented in the literature. They may be prepared from a monomer blend that comprises water soluble ethylenically unsaturated monomers and polymerised by any suitable polymerisation technique that provides microparticles which have an unswollen particle diameter of less than 750 nanometers. The monomer blend may also comprise cross-linking agent. Generally the amount of crosslinking agent may be any suitable amount, for instance up to 50,000 ppm on a molar basis. Typically the amounts of cross-linking agent are in the range 1 to 5,000 ppm.

The microparticles may be prepared in accordance with the teachings of EP-A-484617. Desirably the microparticles exhibit a solution viscosity of at least 1.1 mPa.s and a cross-linking agent content of above 4 molar ppm based on monomeric units. Preferably the microparticles have an ionicity of at least 5.0% More preferably the microparticles are anionic.

In one form of the invention the microparticles are microbeads prepared in accordance with EP462365. The

microbeads have a particle size of less than 750 nanometers if cross-linked and less than 60 nanometers if non-cross-linked and water-insoluble.

Preferably the microparticles exhibit a rheological oscillation value of tan delta at 0.005 Hz of below 0.7 based on 1.5% by weight polymer concentration in water. More preferably the tan delta value is below 0.5 and usually in the range 0.1 to 0.3.

It has surprisingly been found that flocculating the cellulosic suspension using a flocculation system that comprises a siliceous material and organic polymeric microparticles provides improvements in retention, drainage and formation by comparison to a system using the polymeric microparticles alone or the siliceous material in the absence of the polymeric microparticles.

The siliceous material may be any of the materials selected from the group consisting of silica based particles, silica microgels, colloidal silica, silica sols, silica gels, polysilicates, aluminosilicates, polyaluminosilicates, borosilicates, polyborosilicates, zeolites or swellable clay.

This siliceous material may be in the form of an anionic microparticulate material. Alternatively the siliceous material may be a cationic silica. Desirably the siliceous material may be selected from silicas and polysilicates. The silica may be for example any colloidal silica, for instance as described in WO-A-8600100. The polysilicate may be a colloidal silicic acid as described in U.S. Pat. No. 4,388,150.

The polysilicates of the invention may be prepared by acidifying an aqueous solution of an alkali metal silicate. For instance polysilicic microgels otherwise known as active silica may be prepared by partial acidification of alkali metal silicate to about pH 8-9 by use of mineral acids or acid exchange resins, acid salts and acid gases. It may be desired to age the freshly formed polysilicic acid in order to allow sufficient three dimensional network structure to form. Generally the time of ageing is insufficient for the polysilicic acid to gel. Particularly preferred siliceous material include polyalumino-silicates. The polyaluminosilicates may be for instance aluminated polysilicic acid, made by first forming polysilicic acid microparticles and then post treating with aluminium salts, for instance as described in U.S. Pat. No. 5,176,891. Such polyaluminosilicates consist of silicic microparticles with the aluminium located preferentially at the surface.

Alternatively the polyaluminosilicates may be polyparticulate polysilicic microgels of surface area in excess of 1000 m<sup>2</sup>/g formed by reacting an alkali metal silicate with acid and water soluble aluminium salts, for instance as described in U.S. Pat. No. 5,482,693. Typically the polyaluminosilicates may have a mole ratio of alumina:silica of between 1:10 and 1:1500.

Polyaluminosilicates may be formed by acidifying an aqueous solution of alkali metal silicate to pH 9 or 10 using concentrated sulphuric acid containing 1.5 to 2.0% by weight of a water soluble aluminium salt, for instance aluminium sulphate. The aqueous solution may be aged sufficiently for the three dimensional microgel to form. Typically the polyaluminosilicate is aged for up to about two and a half hours before diluting the aqueous polysilicate to 0.5 weight % of silica.

The siliceous material may be a colloidal borosilicate, for instance as described in WO-A-9916708. The colloidal borosilicate may be prepared by contacting a dilute aqueous solution of an alkali metal silicate with a cation exchange resin to produce a silicic acid and then forming a heel by mixing together a dilute aqueous solution of an alkali metal

borate with an alkali metal hydroxide to form an aqueous solution containing 0.01 to 30% B<sub>2</sub>O<sub>3</sub>, having a pH of from 7 to 10.5.

The swellable clays may for instance be typically a bentonite type clay. The preferred clays are swellable in water and include clays which are naturally water swellable or clays which can be modified, for instance by ion exchange to render them water swellable. Suitable water swellable clays include but are not limited to clays often referred to as hectorite, smectites, montmorillonites, nontronites, saponite, sauconite, hormites, attapulgites and sepiolites. Typical anionic swelling clays are described in EP-A-235893 and EP-A-335575.

Most preferably the clay is a bentonite type clay. The bentonite may be provided as an alkali metal bentonite. Bentonites occur naturally either as alkaline bentonites, such as sodium bentonite or as the alkaline earth metal salt, usually the calcium or magnesium salt. Generally the alkaline earth metal bentonites are activated by treatment with sodium carbonate or sodium bicarbonate. Activated swellable bentonite clay is often supplied to the paper mill as dry powder. Alternatively the bentonite may be provided as a high solids flowable slurry, for example at least 15 or 20% solids, for instance as described in EP-A485124, WO-A-9733040 and WO-A-9733041.

The microparticles may be made as microemulsions by a process employing an aqueous solution comprising a cationic or anionic monomer and crosslinking agent; an oil comprising a saturated hydrocarbon; and an effective amount of a surfactant sufficient to produce particles of less than about 0.75 micron in unswollen number average particle size diameter. Microbeads are also made as microgels by procedures described by Ying Huang et. al., *Makromol. Chem.* 186, 273-281 (1985) or may be obtained commercially as microlatices. The term "microparticle", as used herein, is meant to include all of these configurations, i.e. beads per se, microgels and microlatices.

Polymerisation of the emulsion to provide microparticles may be carried out by adding a polymerization initiator, or by subjecting the emulsion to ultraviolet radiation. An effective amount of a chain transfer agent may be added to the aqueous solution of the emulsion, so as to control the polymerization. It was surprisingly found that the crosslinked, organic, polymeric microparticles have a high efficiency as retention and drainage aids when their particle size is less than about 750 nm in diameter and preferably less than about 300 nm in diameter and that the noncrosslinked, organic, water-insoluble polymer microparticles have a high efficiency when their size is less than about 60 nm. The efficiency of the crosslinked microparticles at a larger size than the noncrosslinked microparticles may be attributed to the small strands or tails that protrude from the main crosslinked polymer.

Cationic microparticles used herein include those made by polymerizing such monomers as diallyldialkylammonium halides; acryloxyalkyltrimethylammonium chloride; (meth)acrylates of dialkylaminoalkyl compounds, and salts and quaternaries thereof and, monomers of N,N-dialkylaminoalkyl(meth)acrylamides, and salt and quaternaries thereof, such as N,N-dimethyl aminoethylacrylamides; (meth)acrylamidopropyltrimethylammonium chloride and the acid or quaternary salts of N,N-dimethylaminoethylacrylate and the like. Cationic monomers which may be used herein are of the following general formulae:



where  $R_1$  is hydrogen or methyl,  $R_2$  is hydrogen or lower alkyl of  $C_1$  to  $C_4$ ,  $R_3$  and/or  $R_4$  are hydrogen, alkyl of  $C_1$  to  $C_{12}$ , aryl, or hydroxyethyl and  $R_2$  and  $R_3$  or  $R_2$  and  $R_4$  can combined to form a cyclic ring containing one or more hetero atoms,  $Z$  is the conjugate base of an acid,  $X$  is oxygen or  $—NR_1$  wherein  $R_1$  is as defined above, and  $A$  is an alkylene group of  $C_1$  to  $C_{12}$ ; or



where  $R_5$  and  $R_6$  are hydrogen or methyl,  $R_7$  is hydrogen or alkyl of  $C_1$  to  $C_{12}$  and  $R_8$  is hydrogen, alkyl of  $C_1$  to  $C_{12}$ , benzyl or hydroxyethyl; and  $Z$  is as defined above.

Anionic microparticles that are useful herein those made by hydrolyzing acrylamide polymer microparticles etc. those made by polymerizing such monomers as (methyl) acrylic acid and their salts, 2-acrylamido-2-methylpropane sulfonate, sulfoethyl-(meth)acrylate, vinylsulfonic acid, styrene sulfonic acid, maleic or other dibasic acids or their salts or mixtures thereof.

Nonionic monomers, suitable for making microparticles as copolymers with the above anionic and cationic monomers, or mixtures thereof, include (meth)acrylamide; N-alkyacrylamides, such as N-methylacrylamide; N,N-dialkylacrylamides, such as N,N-dimethylacrylamide; methyl acrylate; methyl methacrylate; acrylonitrile; N-vinyl methylacetamide; N-vinyl methyl formamide; vinyl acetate; N-vinyl pyrrolidone, mixtures of any of the foregoing and the like.

These ethylenically unsaturated, non-ionic monomers may be copolymerized, as mentioned above, to produce cationic, anionic or amphoteric copolymers. Preferably, acrylamide is copolymerized with an ionic and/or cationic monomer. Cationic or anionic copolymers useful in making microparticles comprise from about 0 to about 99 parts, by weight, of non-ionic monomer and from about 100 to about 1 part, by weight, of cationic or anionic monomer, based on the total weight of the anionic or cationic and non-ionic monomers, preferably from about 10 to about 90 parts, by weight, of non-ionic monomer and about 10 to about 90 parts, by weight, of cationic or anionic monomer, same basis i.e. the total ionic charge in the microparticle must be greater than about 1%. Mixtures of polymeric microparticles may also be used if the total ionic charge of the mixture is also over about 1%. Most preferably, the microparticles contain from about 20 to 80 parts, by weight, of non-ionic monomer and about 80 to about 20 parts by weight, same basis, of cationic or anionic monomer or mixture thereof. Polymerization of the monomers occurs in the presence of a poly-functional crosslinking agent to form the cross-linked micro-particle. Useful polyfunctional crosslinking agents comprise compounds having either at least two double bounds, a double bond and a reactive group, or two reactive groups. Illustrative of those containing at least two double bounds are N,N-methylenebisacrylamide; N,N-

methylenebismethacrylamide; polyethyleneglycol diacrylate; polyethyleneglycol dimethacrylate; N-vinyl acrylamide; divinylbenzene; triallylammonium salts, N-methylallylacrylamide and the like. Polyfunctional branching agents containing at least one double bond and at least one reactive group include glycidyl acrylate; glycidyl methacrylate; acrolein; methylolacrylamide and the like. Polyfunctional branching agents containing at least two reactive groups include dialdehydes, such as glyoxal; diepoxy compounds; epichlorohydrin and the like.

10 oxy compounds, phenol-formaldehyde and the like.

Crosslinking agents are to be used in sufficient quantities to assure a cross-linked composition. Preferably, at least about 4 molar parts per million of crosslinking agent based on the monomeric units present in the polymer are employed to induce sufficient crosslinking and especially preferred is a crosslinking agent content of from about 4 to about 6000 molar parts per million, preferably, about 20-4000. More preferably the amount of crosslinking agents used is in excess of 60 or 70 molar ppm. The amounts particularly preferred are in excess of 100 or 150 ppm, especially in the 15 range 200 to 1000 ppm. Most preferably the amount of cross-linking agents is in the range 350 to 750 ppm.

The polymeric microparticles of this invention are preferably prepared by polymerization of the monomers in an emulsion as disclosed in application, EP-484617. Polymerization in microemulsions and inverse emulsions may be used as is known to those skilled in this art. P. Speiser reported in 1976 and 1977 a process for making spherical "nanoparticles" with diameters less than 800 Ångstrom by (1) solubilizing monomers, such as acrylamide and 25 methylenebisacrylamide, in micelles and (2) polymerizing the monomers, See J. Pharm. Sa., 65(12), 1763 (1976) and U.S. Pat. No. 4,021,364. Both inverse water-in-oil and oil-in-water "nanoparticles" were prepared by this process. 30 While not specifically called microemulsion polymerization 35 by the author, this process does contain all the features which are currently used to define microemulsion polymerization. These reports also constitute the first examples of polymerization of acrylamide in a microemulsion. Since then, numerous publications reporting polymerization of 40 hydrophobic monomers in the oil phase of microemulsions have appeared. See, for examples, U.S. Pat. Nos. 4,521,317 and 4,681,912; Stoffer and Bone, J. Dispersion Sci. and Tech., 1(1), 37, 1980; and Atik and Thomas, J. Am. Chem. Soc., 103 (14), 4279 (1981); and GB 2161492A.

See, 103 (1), 127 (1981), and GB 2101722A.

45 The cationic and/or anionic emulsion polymerization process is conducted by (i) preparing a monomer emulsion by adding an aqueous solution of the monomers to a hydrocarbon liquid containing appropriate surfactant or surfactant mixture to form an inverse monomer emulsion consisting of

50 small aqueous droplets which, when polymerized, result in polymer particles of less than 0.75 micron in size, dispersed in the continuous oil phase and (ii) subjecting the monomer microemulsion to free radical polymerization.

The aqueous phase comprises an aqueous mixture of the 55 cationic and/or anionic monomers and optionally, a non-  
ionic monomer and the crosslinking agent, as discussed  
above. The aqueous monomer mixture may also comprise  
such conventional additives as are desired. For example, the  
mixture may contain chelating agents to remove polymer-  
ization inhibitors, pH adjusters, initiators and other conven-  
tional additives.

Essential to the formation of the emulsion, which may be defined as a swollen, transparent and thermodynamically stable emulsion comprising two liquids insoluble in each other and a surfactant, in which the micelles are less than 0.75 micron in diameter, is the selection of appropriate organic phase and surfactant.

The selection of the organic phase has a substantial effect on the minimum surfactant concentration necessary to obtain the inverse emulsion. The organic phase may comprise a hydrocarbon or hydrocarbon mixture. Saturated hydrocarbons or mixtures thereof are the most suitable in order to obtain inexpensive formulations. Typically, the organic phase will comprise benzene, toluene, fuel oil, kerosene, odorless mineral spirits or mixtures of any of the foregoing.

The ratio, by weight, of the amounts of aqueous and hydrocarbon phases is chosen as high as possible, so as to obtain, after polymerization, an emulsion of high polymer content. Practically, this ratio may range, for example for about 0.5 to about 3:1, and usually approximates about 1:1, respectively.

One or more surfactants may be selected in order to obtain HLB (Hydrophilic Lipophilic Balance) value ranging from about 8 to about 11. In addition to the appropriate HLB value, the concentration of surfactant must also be optimized, i.e. sufficient to form an inverse emulsion. Too low a concentration of surfactant leads to inverse emulsions of the prior art and too high a concentrations results in undue costs. Typical surfactants useful, in addition to those specifically discussed above, may be anionic, cationic or non-ionic and may be selected from polyoxyethylene (20) sorbitan trioleate, sorbitan trioleate, sodium di-2-ethylhexylsulfosuccinate, oleamidopropylidimethylamine; sodium isostearyl-2-lactate and the like. Polymerization of the emulsion may be carried out in any manner known to those skilled in the art. Initiation may be effected with a variety of thermal and redox free-radical initiators including azo compounds, such as azobisisobutyronitrile; peroxides, such as t-butyl peroxide; inorganic compounds, such as potassium persulfate and redox couples, such as ferrous ammonium sulfate/ammonium persulfate. Polymerization may also be effected by photochemical irradiation processes, irradiation, or by ionizing radiation with a  $\text{Co}^{60}$  source. Preparation of an aqueous product from the emulsion may be effected by inversion by adding it to water which may contain a breaker surfactant. Optionally, the polymer may be recovered from the emulsion by stripping or by adding the emulsion to a solvent which precipitates the polymer, e.g. isopropanol, filtering off the resultant solids, drying and redispersing in water.

The high molecular weight, ionic, synthetic polymers used in the present invention preferably have a molecular weight in excess of 100,000 and preferably between about 250,000 and 25,000,000. Their anionicity and/or cationicity may range from 1 mole percent to 100 mole percent. The ionic polymer may also comprise homopolymers or copolymers of any of the ionic monomers discussed above with regard to the ionic beads, with acrylamide copolymers being preferred.

The tan delta at 0.005 Hz value is obtained using a Controlled Stress Rheometer in Oscillation mode on a 1.5% by weight aqueous solution of polymer in deionised water after tumbling for two hours. In the course of this work a Carrimed CSR 100 is used fitted with a 6 cm acrylic cone, with a  $1^\circ 58'$  cone angle and a  $58 \mu\text{m}$  truncation value (Item ref 5664). A sample volume of approximately 2–3 cc is used. Temperature is controlled at  $20.0^\circ \text{C} \pm 0.1^\circ \text{C}$ . using the Peltier Plate. An angular displacement of  $5 \pm 10^{-4}$  radians is employed over a frequency sweep from 0.005 Hz to 1 Hz in 12 stages on a logarithmic basis.  $G'$  and  $G''$  measurements are recorded and used to calculate tan delta ( $G''/G'$ ) values. The value of tan delta is the ratio of the loss (viscous) modulus  $G''$  to storage (elastic) modulus  $G'$  within the system.

At low frequencies (0.005 Hz) it is believed that the rate of deformation of the sample is sufficiently slow to enable linear or branched entangled chains to disentangle. Network or cross-linked systems have permanent entanglement of the chains and show low values of tan delta across a wide range of frequencies. Therefore low frequency (e.g. 0.005 Hz) measurements are used to characterise the polymer properties in the aqueous environment.

According to the invention the components of the flocculation system may be combined into a mixture and introduced into the cellulosic suspension as a single composition. Alternatively the polymeric microparticles and the siliceous material may be introduced separately but simultaneously. Preferably, however, the siliceous material and the polymeric microparticles are introduced sequentially more preferably when the siliceous material is introduced into the suspension and then the polymeric microparticles.

In a preferred form of the invention the process comprises including a further flocculating material into the cellulosic suspension before adding the polymeric microparticles and siliceous material. The further flocculating material may be anionic, non-ionic or cationic. It may be for instance a synthetic or natural polymer and may be a water soluble substantially linear or branched polymer. Alternatively the first flocculating material is a cross-linked polymer or a blend of cross-linked and water soluble polymer. In a preferred form of the invention the polymeric microparticles and siliceous material are added to the cellulosic suspension, which suspension has been pre-treated with a cationic material. The cationic pre-treatment may be by incorporating cationic materials into the suspension at any point prior to the addition of the polymeric microparticle and siliceous material.

Thus the cationic treatment may be immediately before adding the polymeric microparticle and siliceous material although preferably the cationic material is introduced into the suspension sufficiently early in order for it to be distributed throughout the cellulosic suspension before either the polymeric microparticle or siliceous material are added. It may be desirable to add the cationic material before one of the mixing, screening or cleaning stages and in some instances before the stock suspension is diluted. It may even be beneficial to add the cationic material into the mixing chest or blend chest or even into one or more of the components of the cellulosic suspension, for instance, coated broke or filler suspensions for instance precipitated calcium carbonate slurries.

The cationic material may be any number of cationic species such as water soluble cationic organic polymers, or inorganic materials such as alum, polyaluminium chloride, aluminium chloride trihydrate and aluminochloro hydrate. The water soluble cationic organic polymers may be natural polymers, such as cationic starch or synthetic cationic polymers. Particularly preferred are cationic materials that coagulate or flocculate the cellulosic fibres and other components of the cellulosic suspension.

According to another preferred aspect of the invention the flocculation system comprises at least three flocculent components. Thus this preferred system employs polymeric microparticles, siliceous material and at least one additional flocculant/coagulant.

The additional flocculant/coagulant component is preferably added prior to either the siliceous material or polymeric microparticle. Typically the additional flocculent is a natural or synthetic polymer or other material capable of causing flocculation/coagulation of the fibres and other components of the cellulosic suspension. The additional flocculant/

coagulant may be a cationic, non-ionic, anionic or amphoteric natural or synthetic polymer. It may be a natural polymer such as natural starch, cationic starch, anionic starch or amphoteric starch. Alternatively it may be any water soluble synthetic polymer which preferably exhibits ionic character. The preferred ionic water soluble polymers have cationic or potentially cationic functionality. For instance the cationic polymer may comprise free amine groups which become cationic once introduced into a 10 cellulosic suspension with a sufficiently low pH so as to protonate free amine groups. Preferably however, the cationic polymers carry a permanent cationic charge, such as quaternary ammonium groups.

The additional flocculant/coagulant may be used in addition to the cationic pre-treatment step described above. In a particularly preferred system the cationic pre-treatment is also the additional flocculant/coagulant. Thus this preferred process comprises adding a cationic flocculant/coagulant to the cellulosic suspension or to one or more of the suspension components thereof, in order to cationically pre-treat the cellulosic suspension. The suspension is subsequently subjected to further flocculation stages comprising addition of the polymeric microparticles and the siliceous material.

The cationic flocculant/coagulant is desirably a water soluble polymer which may for instance be a relatively low molecular weight polymer of relatively high cationicity. For instance the polymer may be a homopolymer of any suitable ethylenically unsaturated cationic monomer polymerised to provide a polymer with an intrinsic viscosity of up to 3 dl/g. Homopolymers of diallyl dimethyl ammonium chloride are preferred. The low molecular weight high cationicity polymer may be an addition polymer formed by condensation of amines with other suitable di- or tri-functional species. For instance the polymer may be formed by reacting one or more amines selected from dimethyl amine, trimethyl amine and ethylene diamine etc and epihalohydrin, epichlorohydrin being preferred. Preferably the cationic flocculant/coagulant is a polymer that has been formed from a water soluble ethylenically unsaturated cationic monomer or blend of monomers wherein at least one of the monomers in the blend is cationic or potentially cationic. By water soluble we mean that the monomer has a solubility in water of at least 5 g/100 cc. The cationic monomer is preferably selected from diallyl di alkyl ammonium chlorides, acid addition salts or quaternary ammonium salts of either dialkyl amino alkyl (meth) acrylate or dialkyl amino alkyl (meth) acrylamides. The cationic monomer may be polymerised alone or copolymerised with water soluble non-ionic, cationic or anionic monomers. More preferably such polymers have an intrinsic viscosity of at least 3 dl/g, for instance as high as 16 or 18 dl/g, but usually in the range 7 or 8 to 14 or 15 dl/g.

Particularly preferred cationic polymers include copolymers of methyl chloride quaternary ammonium salts of dimethylaminoethyl acrylate or methacrylate. The water soluble cationic polymer may be a polymer with a Theological oscillation value of tan delta at 0.005 Hz of above 1.1 (defined by the method given herein) for instance as provided for in copending patent application based on the priority U.S. patent application Ser. No. 60/164,231 (reference PP/W-21916/P1/AC 526).

The water soluble cationic polymer may also have a slightly branched structure for instance by incorporating small amounts of branching agent e.g. up to 20 ppm by weight. Such branched polymers may also be prepared by including a chain transfer agent into the monomer mix. The chain transfer agent may be included in an amount of at least 2 ppm by weight and may be included in an amount of up

to 200 ppm by weight. Typically the amounts of chain transfer agent are in the range 10 to 50 ppm by weight. The chain transfer agent may be any suitable chemical substance, for instance sodium hypophosphite, 2-mercaptoethanol, 5 malic acid or thioglycolic acid.

When the flocculation system comprises cationic polymer, it is generally added in an amount sufficient to effect flocculation. Usually the dose of cationic polymer would be above 20 ppm by weight of cationic polymer based 10 on dry weight of suspension. Preferably the cationic polymer is added in an amount of at least 50 ppm by weight for instance 100 to 2000 ppm by weight. Typically the polymer dose may be 150 ppm to 600 ppm by weight, especially between 200 and 400 ppm.

Typically the amount of polymeric microparticle may be at least 20 ppm by weight based on weight of dry suspension, although preferably is at least 50 ppm by weight, particularly between 100 and 2000 ppm by weight. Doses of between 150 and 600 ppm by weight are more preferred, especially between 200 and 400 ppm by weight. The siliceous material may be added at a dose of at least 100 ppm by weight based on dry weight of suspension. Desirably the dose of siliceous material may be in the range of 500 or 750 ppm to 10,000 ppm by weight. Doses of 1000 to 2000 20 ppm by weight siliceous material have been found to be most effective.

In one preferred form of the invention the cellulosic suspension is subjected to mechanical shear following addition of at least one of the components of the flocculating 30 system. Thus in this preferred form at least one component of the flocculating system is mixed into the cellulosic suspension causing flocculation and the flocculated suspension is then mechanically sheared. This shearing step may be achieved by passing the flocculated suspension through one or more shear stages, selected from pumping, cleaning or mixing stages. For instance such shearing stages include fan pumps and centri-screens, but could be any other stage in the 35 process where shearing of the suspension occurs.

The mechanical shearing step desirably acts upon the 40 flocculated suspension in such a way as to degrade the flocs. All of the components of the flocculating system may be added prior to a shear stage although preferably at least the last component of the flocculating system is added to the cellulosic suspension at a point in the process where there is 45 no substantial shearing before draining to form the sheet. Thus it is preferred that at least one component of the flocculating system is added to the cellulosic suspension and the flocculated suspension is then subjected to mechanical shear wherein the flocs are mechanically degraded and then 50 at least one component of the flocculating system is added to reflocculate the suspension prior to draining.

According to a more preferred form of the invention the water-soluble cationic polymer is added to the cellulosic suspension and then the suspension is then mechanically sheared. The siliceous material and the polymeric microparticle are then added to the suspension. The polymeric microparticle and siliceous material may be added either as a premixed composition or separately but simultaneously but preferably they are added sequentially. Thus the suspension may be re-flocculated by addition of the polymeric microparticles followed by the siliceous material but preferably the suspension is reflocculated by adding siliceous material and then the polymeric microparticles.

The first component of the flocculating system may be 65 added to the cellulosic suspension and then the flocculated suspension may be passed through one or more shear stages. The second component of the flocculation system may be

added to re-flocculate the suspension, which re-flocculated suspension may then be subjected to further mechanical shearing. The sheared reflocculated suspension may also be further flocculated by addition of a third component of the flocculation system. In the case where the addition of the components of the flocculation system is separated by shear stages it is preferred that the polymeric microparticle component is the last component to be added.

In another form of the invention the suspension may not be subjected to any substantial shearing after addition of any of the components of the flocculation system to the cellulosic suspension. The siliceous material, polymeric microparticle and where included the water soluble cationic polymer may all be introduced into the cellulosic suspension after the last shear stage prior to draining. In this form of the invention the polymeric microparticle may be the first component followed by either the cationic polymer (if included) and then the siliceous material. However, other orders of addition may also be used.

In a further preferred form of the invention we provide a process of making paper or board in which the a cationic material is introduced into the furnish or components thereof and the treated furnish is passed through at least one shear stage selected from mixing, cleaning and screening stages and then the furnish is subjected to flocculation by a flocculation system comprising anionic polymeric microparticles and a siliceous material. As given before the anionic polymeric microparticles and siliceous material may be added simultaneously or added sequentially. When added sequentially there may be a shear stage between the addition points.

A particularly preferred process employs the organic microparticle as the major component of the total flocculation system comprising a siliceous material and organic microparticles. Hence the organic microparticle should in this case be greater than 50%, preferably greater than 55% of the total flocculation system. In this form of the invention it is highly desirable that the ratio of organic microparticles to siliceous material is in the range 55:45 and 99:1 based on weight of materials. Preferably the ratio of organic microparticle to siliceous material is between 60:40 and 90:10, more preferably between 65:35 and 80:20, especially about 75:25.

In one preferred form of the invention we provide a process of preparing paper from a cellulosic stock suspension comprising filler. The filler may be any of the traditionally used filler materials. For instance the filler may be clay such as kaolin, or the filler may be a calcium carbonate which could be ground calcium carbonate or in particular precipitated calcium carbonate, or it may be preferred to use titanium dioxide as the filler material. Examples of other filler materials also include synthetic polymeric fillers. Generally a cellulosic stock comprising substantial quantities of filler are more difficult to flocculate. This is particularly true of fillers of very fine particle size, such as precipitated calcium carbonate.

Thus according to a preferred aspect of the present invention we provide a process for making filled paper. The paper making stock may comprise any suitable amount of filler. Generally the cellulosic suspension comprises at least 5% by weight filler material. Typically the amount of filler will be up to 40%, preferably between 10% and 40% filler. Thus according to this preferred aspect of this invention we provide a process for making filled paper or paper board wherein we first provide a cellulosic suspension comprising filler and in which the suspension solids are flocculated by introducing into the suspension a flocculating system com-

prising a siliceous material and polymeric microparticle as defined herein.

In an alternative form of the invention we provide a process of preparing paper or paperboard from a cellulosic stock suspension which is substantially free of filler.

As an illustration of the invention a cellulosic stock is prepared containing a 50/50 bleached birch/bleached pine suspension containing 40% by weight (on total solids) precipitated calcium carbonate. The stock suspension is beaten to a freeness of 55° (Schopper Riegler method) before the addition of filler. 5 kg per tonne (on total solids) cationic starch (0.045 DS) is added to the suspension.

500 grams per tonne of copolymer of acrylamide with methyl chloride quaternary ammonium salt of dimethylaminooethyl acrylate (75/25 wt./wt.) of intrinsic viscosity above 11.0 dl/g is mixed with the stock and then after shearing the stock using a mechanical stirrer then 250 grams per tonne of a polymeric microparticle comprising anionic copolymer of acrylamide with sodium acrylate (65/35) (wt./wt.) with 700 ppm by weight methylene bis acrylamide prepared by microemulsion polymerisation as given herein is mixed into the stock. 2000 grams per tonne of an aqueous colloidal silica is applied after the shearing but immediately prior to the addition of polymeric microparticle.

We find that for doses that provide equivalent drainage and/or retention the combination of both microparticle and silica gives improved formation over the separate use of microparticle or silica.

The following Example further illustrate the invention without in any way being intended to limit the invention.

#### EXAMPLE 1

A model fine paper stock is prepared containing a fibre content comprising equal mix of bleached birch and bleached pine and contained 40%, by weight (PCC on dry fibre), precipitated calcium carbonate (Albacar HO, Specialty Minerals Inc). The stock is used at a 1% paper stock concentration.

The following ADDITIVES are used in the evaluation  
**CATIONIC POLYMER**=High molecular copolymer of acrylamide with dimethylaminooethyl acrylate, methyl chloride quaternary ammonium salt (60/40 weight/weight) then made up as a 0.1% solution.

**ORGANIC-MICROPARTICLE**=Anionic copolymer of acrylamide with sodium acrylate (65/35) (wt./wt.) with 300 ppm by weight methylene bis acrylamide prepared by microemulsion polymerisation as given herein, then made up in water as a 0.1% polymer concentration.

**Bentonite**=A commercially available bentonite clay—made up as a 0.1% solids by weight aqueous suspension using deionised water.

The single component systems are evaluated by adding the ADDITIVE at the stated dose to 500 ml of the paper stock suspension in a 500 ml measuring cylinder and mixed by 5 hand inversions before being transferred to the DDJ with the stirrer set at 1000 rpm. The tap was opened after 5 seconds and then closed after a further 15 seconds. 250 ml of filtrate is collected for each test.

The dual component systems were evaluated by adding the CATIONIC POLYMER at a dose of 250 grams per tonne to the stock in a measuring cylinder and mixing by five hand inversions. The flocculated stock is then transferred to a shear pot and mixed for 30 seconds with a Heidolph stirrer at a speed of 1500 rpm. The sheared stock was then returned to the measuring cylinder before being dosed with the required amount of anionic component. The re-flocculated

suspension was transferred to the DDJ with the stirrer set at 1000 rpm and the filtrate was collected in the same way as specified above.

The three component system are evaluated in the same way as the dual component systems except that the ORGANIC MICROPARTICLE is added immediately after the BENTONITE addition and then mixed by hand inversions.

The blank (no chemical addition) retention value is also determined. For the blank retention, the stock is added to the DDJ, with the stirrer set at 1000 rpm, and the filtrate is collected as above.

A Schopper-Riegler free drainage survey is carried out using the same flocculation systems as described in the method for the retention survey.

#### First Pass Retention

All retention values shown are percentages

The blank retention is 65.1%

#### Single Addition Test

TABLE 1

| Dose Level (g/t) | ORGANIC MICROPARTICLE |
|------------------|-----------------------|
| 125              | 61.7                  |
| 250              | 63.7                  |
| 500              | 66.2                  |
| 750              | 66.9                  |

#### Dual Component

##### CATIONIC POLYMER used at 250 g/t

TABLE 2

| Dose Level (g/t) | ORGANIC-MICROPARTICLE | BENTONITE |
|------------------|-----------------------|-----------|
| 0                | 62.7                  | 62.7      |
| 125              | 71.5                  | 64.1      |
| 250              | 74.5                  | 66.8      |
| 500              | 76.2                  | 70.8      |
| 750              | 78.9                  | 72.5      |

#### Three Component System

##### CATIONIC POLYMER used at 250 g/t

##### BENTONITE used at 500 g/t

TABLE 3

| Dose Level (g/t) | ORGANIC-MICROPARTICLE |
|------------------|-----------------------|
| 0                | 70.8                  |
| 125              | 78.8                  |
| 250              | 82.0                  |
| 500              | 84.7                  |
| 750              | 84.5                  |

The results of table 3 show the benefits of using both siliceous material and organic microparticle.

#### Filer Retention

All retention values shown are percentages

The blank filler retention is 31.3%

#### Single Addition Test

TABLE 4

| Dose Level (g/t) | ORGANIC MICROPARTICLE |
|------------------|-----------------------|
| 125              | 23.7                  |
| 250              | 29.1                  |
| 500              | 36.1                  |
| 750              | 36.6                  |

#### Dual Component

##### CATIONIC POLYMER used at 250 g/t

TABLE 5

| Dose Level (g/t) | ORGANIC-MICROPARTICLE | BENTONITE |
|------------------|-----------------------|-----------|
| 0                | 26.7                  | 26.7      |
| 125              | 45.7                  | 29.1      |
| 250              | 51.5                  | 35.6      |
| 500              | 55.3                  | 43.2      |
| 750              | 60.8                  | 46.6      |

#### Three Component System

##### CATIONIC POLYMER used at 250 g/t

##### BENTONITE used at 500 g/t

TABLE 6

| Dose Level (g/t) | ORGANIC-MICROPARTICLE |
|------------------|-----------------------|
| 0                | 43.2                  |
| 125              | 60.2                  |
| 250              | 66.9                  |
| 500              | 72.2                  |
| 750              | 72.2                  |

The results of table 6 show the benefits in terms of filler retention of using both siliceous material and organic microparticle.

#### Free Drainage

The free drainage results are measured in seconds for 600 ml of filtrate to be collected. The blank free drainage is 104 seconds

#### Single Addition Test

TABLE 7

| Dose Level (g/t) | ORGANIC MICROPARTICLE |
|------------------|-----------------------|
| 125              | 114                   |
| 250              | 130                   |
| 500              | 156                   |
| 750              | 155                   |

15

Dual Component

CATIONIC POLYMER used at 250 g/t

TABLE 8

| Dose Level (g/t) | ORGANIC-MICROPARTICLE | BENTONITE |
|------------------|-----------------------|-----------|
| 0                | 78                    | 78        |
| 125              | 41                    | 52        |
| 250              | 39                    | 40        |
| 500              | 44                    | 31        |
| 750              | 46                    | 28        |

Three Component System

CATIONIC POLYMER used at 250 g/t

BENTONITE used at 500 g/t

TABLE 9

| Dose Level (g/t) | ORGANIC-MICROPARTICLE |
|------------------|-----------------------|
| 0                | 31                    |
| 125              | 23                    |
| 250              | 21                    |
| 500              | 20                    |
| 750              | 23                    |

The results of table 9 show the benefits of using both 30 siliceous material and organic microparticle.

## EXAMPLE 2

The First Pass Retention tests of Example 1 are repeated 35 except using an ORGANIC-MICROPARTICLE that has been prepared using 1000 ppm by weight methylene-bis-acrylamide.

## First Pass Retention

All retention values shown are percentages

The blank retention is 82.6%

## Single Addition Test

TABLE 10

| Dose Level (g/t) | CATIONIC POLYMER |
|------------------|------------------|
| 250              | 86.3             |
| 500              | 85.8             |

Dual Component

CATIONIC POLYMER used at 500 g/t

TABLE 11

| Dose Level (g/t) | ORGANIC-MICROPARTICLE | BENTONITE |
|------------------|-----------------------|-----------|
| 0                | 85.8                  | 85.8      |
| 250              | 87.9                  | 82.2      |
| 500              | 87.4                  | 86.7      |

16

Three Component System

CATIONIC POLYMER used at 500 g/t

BENTONITE used at 500 g/t

5

TABLE 12

| Dose Level (g/t) | ORGANIC-MICROPARTICLE |
|------------------|-----------------------|
| 0                | 86.7                  |
| 125              | 89.7                  |
| 250              | 88.3                  |
| 500              | 92.3                  |

The results of table 12 show the benefits of using both 15 siliceous material and organic microparticle.

## EXAMPLE 3

Laboratory headbox stock was prepared to 0.64% consistency with 50% hardwood fibre and 50% softwood fibre and containing 30% precipitated calcium carbonate (PCC) based 20 on dry fibre.

The additives used are as in Example 1 except that the bentonite is replaced by a commercially available polyaluminosilicate microgel (Particol BX<sup>RTM</sup>)

25

## Single Component

A 500 ml aliquot of stock was treated for each retention test; 1000 ml was treated for free drainage testing. For single component testing, the stock was mixed at 1500 rpm for 20 seconds in a Britt jar fixed with an 80M screen. CATIONIC POLYMER was added and, after an additional 5 seconds of shear at 1000 rpm, 100 ml of whitewater was collected through the jar valve for first pass retention testing.

## Two Component System

For the two component systems, CATIONIC POLYMER was added 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330

ticle as the final component in the three-component system with microgel Particol BX.

#### First Pass Ash Retention

Similar trends in first pass ash retention performance are shown in FIG. 2 for the same systems used with Particol BX. The advantage in ash retention is demonstrated by the addition of Organic microparticle to the Particol system.

#### Free Drainage

FIG. 3 shows the free drainage performance of the micro-particle systems tested.

Example 3 demonstrates the improvements over the two component systems using cationic polymer a polysilicate microgel and organic microparticle over the two component systems using cationic polymer and either organic microparticle or polysilicate microgel.

What is claimed is:

1. A process for making paper or paper board comprising forming a cellulosic suspension, flocculating the suspension, draining the suspension on a screen to form a sheet and then drying the sheet,

wherein the suspension is flocculated by adding a flocculation system comprising a siliceous material and organic polymeric microparticles which have an unswollen particle diameter of less than 750 nanometers,

in which the total charge in the organic polymeric microparticle is greater than about 1%, and in which the siliceous material is selected from the group consisting of silica sols, colloidal silica, colloidal silicic acid, polysilicic microgels, aluminated polysilicic acid, polyaluminosilicates consisting of silicic microparticles, silica microgels, polyparticulate polysilicic microgels, colloidal borosilicate, polyborosilicates, cationic silica and swellable clay, wherein the flocculating system comprises,

i) adding up to 400 ppm by weight organic polymeric microparticle and at least 500 ppm by weight of siliceous material, or  
ii) the organic polymeric microparticle and siliceous material is added as a premixed composition.

2. A process according to claim 1 in which the microparticles exhibit a solution viscosity of at least 1.1 mPa.s and a cross-linking agent content of above 4 molar ppm based on monomeric units.

3. A process according to claim 1 in which the microparticles have an ionicity of at least 5.0%.

4. A process according to claim 1 in which the microparticles are microbeads which have a particle size of less than 750 nanometers if cross-linked and less than 60 nanometers if non-cross-linked and water-insoluble.

5. A process according to claim 1 in which the microparticles exhibit a rheological oscillation value of tan delta at 0.005 Hz of below 0.7 based on 1.5% by weight polymer concentration in water.

6. A process according to claims 5 in which the tan delta value is below 0.5.

7. A process according to claim 1 in which the siliceous material is an anionic microparticulate material.

8. A process according to claim 1 in which the siliceous material is a bentonite type clay.

9. A process according to claim 1 in which the siliceous material is selected from the group consisting of hectorite,

smectites, montmorillonites, nontronites, saponite, saucouite, hormites, attapulgites and sepiolites.

10. A process according to claim 1 in which the components of the flocculation system are introduced into the cellulosic suspension sequentially.

11. A process according to claim 1 in which the siliceous material is introduced into the suspension and then the polymeric microparticle is included in the suspension.

12. A process according to claim 1 in which the polymeric microparticle is introduced into the suspension and then the siliceous material is included in the suspension.

13. A process according to claim 1 in which the cellulosic suspension is treated by inclusion of a further flocculating material into the suspension prior to introducing the polymeric microparticle and siliceous material.

14. A process according to claim 13 in which the further flocculating material is a cationic material selected from the group consisting of water soluble cationic organic polymers, inorganic materials such as alum, polyaluminium chloride, aluminium chloride trihydrate and aluminium chloride hydrate.

15. A process according to claim 1 in which the flocculating system additionally comprises at least one additional flocculant/coagulant.

16. A process according to claim 15 in which the flocculant/coagulant is a water soluble polymer.

17. A process according to claim 14 in which the cationic polymer is formed from a water soluble ethylenically unsaturated monomer or water soluble blend of ethylenically unsaturated monomers comprising at least one cationic monomer.

18. A process according to claim 14 in which the cationic polymer is a branched cationic polymer which has an intrinsic viscosity above 3 dl/g and exhibits a rheological oscillation value of tan delta at 0.005 Hz of above 0.7.

19. A process according to claim 14 in which the cationic polymer has an intrinsic viscosity above 3 dl/g and exhibits a rheological oscillation value of tan delta at 0.005 Hz of above 1.1.

20. A process according to claim 1 in which the suspension is subjected to mechanical shear following the addition of at least one of the components of the flocculating system.

21. A process according to claim 1 in which the suspension is first flocculated by introducing the cationic polymer, optionally subjecting the suspension to mechanical shear and then reflocculating the suspension by introducing the polymeric microparticle and siliceous material.

22. A process according to claim 1 in which the cellulosic suspension is reflocculated by introducing the siliceous material and then the polymeric microparticle.

23. A process according to claim 22 in which the cellulosic suspension is reflocculated by introducing the polymeric microparticle and then the siliceous material.

24. A process according to claim 1 in which the cellulosic suspension comprises filler.

25. A process according to claim 24 in which the cellulosic suspension comprises filler in an amount up to 40% by weight based on dry weight of suspension.

26. A process according to claim 24 in which the filler material is selected from precipitated calcium carbonate, ground calcium carbonate, clay and titanium dioxide.

27. A process according to claim 1 in which the cellulosic suspension is substantially free of filler.